# EUROPEAN PATENT SPECIFICATION

(11) **EP 4 334 525 B1**
(45) Date of publication and mention of the grant of the patent: **24.09.2025**
(21) Application number: 22722911.9
(22) Date of filing: 03.05.2022
(51) Int. Cl.: D21C 1/02, D21C 1/04, D21C 3/02, D21C 3/04, D21C 5/00, D21H 11/12

(54) **PROCESS FOR TREATING NON-WOOD FEEDSTOCK**
VERFAHREN ZUR BEHANDLUNG VON NICHTHOLZARTIGEN ROHMATERIALIEN
PROCÉDÉ DE TRAITEMENT DE PRODUIT DE DÉPART NON LIGNEUX

(30) Priority: 03.05.2021 SG 10202104539U
(43) Date of publication of application: 13.03.2024
(73) Proprietor: Asia Pacific Resources International Holdings Ltd., HM11 Hamilton (BM)
(72) Inventor: GINTING, Eduward, Singapore 048624 (SG); ANTES, Rudine, Singapore 048624 (SG); H'NG, Yin Ying, Singapore 048624 (SG); PANDITA, Surya Darma, Singapore 048624 (SG)
(74) Representative: Boult Wade Tennant LLP
(86) International application number: PCT/SG2022/050268
(87) International publication number: WO 2022/235212

(56) References cited:
- EP-A1- 3 339 504
- WO-A1-01/16423
- WO-A1-2006/115310
- WO-A1-2011/126369
- WO-A1-2013/033405
- WO-A1-2013/178608
- WO-A1-2015/108409
- WO-A1-2020/249992
- WO-A1-2021/006798
- CN-B- 108 797 176
- GB-A- 2 534 589
- US-A- 5 433 825
- US-A1- 2010 288 456
- US-A1- 2019 264 388

## Description

The present invention provides methods for pre-treating non-wood empty fruit bunch (EFB) feedstock, a waste product formed after the extraction of palm oil, wherein the pre-treated non-wood feedstock is for subsequent use in producing paper or textile grade pulps for application in industries such as printing writing paper, tissue paper, paper board and fashion garments.

### Background

An increased emphasis on environmental sustainability, coupled with a global shortage of wood feedstock for the pulp and paper industries has meant that focus has shifted towards finding alternative, non-wood feedstock sources. The same is true for the textiles industry where there is a drive towards using renewable raw materials in the production of fibers.

Examples of non-wood feedstocks which provide interesting replacements to wood feedstocks include oil palm empty fruit bunch (EFB) fibers, bamboo, kenaf, wheat/rice straw, coconut coil and bagasse.

Oil palm *(elaeis guineensus),* which is typically grown in Southeast Asian countries such as Indonesia, Malyasia and Thailand, is an important source of vegetable oil, specifically palm oil. Various biomass is produced during the extraction of palm oil. One of the most abundant biomasses produced is Empty Fruit Bunches (EFB) fibers, produced by the first step in the oil extraction process wherein the fruit and nuts are stripped from the fruit bunches. EFB generation is increasing year on year and in 2015 alone, over 30 million tonnes was produced in Indonesia alone. This, in itself, presents an environmental issue as often this waste is simply left to rot and attract rodents.

EFB has a number of properties which make it of interest as a raw material for pulp - it has a high cellulose fiber content and a low lignin content, it resembles hardwood fibers and can be used to provide paper and regenerated cellulose of a high quality. Processes are known in which EFB is used as a raw material which is then subjected to cooking in order to produce chemical pulps from which it is then possible to produce paper and regenerated cellulose, e.g. viscose, modal, lyocell and other man-made cellulose (MMC) fibers.

While EFB and other non-woods are promising replacements for wood in both the paper and textile industries, an issue which arises with these feedstocks is the presence of impurities which cause issues with either processing and/or the quality of the end product. This means that where EFB and other non-woods are used as a feedstock the pulping process needs to be adapted to include pre-treatment steps to remove these impurities. Impurities which are particularly problematic include oils (in the form of fatty acids), silica, ash and other non-process elements (NPEs) content. Although it has been possible to develop processes for the effective removal of oils, ash residue and NPEs, the removal of silica has been found to be difficult.

While difficult with non-wood feedstocks in general, the removal of silica from EFB feedstock is particularly difficult. Investigation of EFB has revealed that it has a particular structure which consists of silica bodies embedded in fiber (see Figure 1) and it is believed that it is these silica bodies which contribute towards the strength and rigidity of EFB (see also Law et al., (2007) Bioresources 2(3), 351-362). However, as described above, the presence of silica in a pulp mill is undesirable for a number of reasons, specifically issues with recovery, poor product quality and damage to machinery as a consequence of silica deposition during processing. Therefore, methods for pre-treating EFB feedstock to remove silica have been investigated. To date, pre-treatment methods have included physical, chemical and biological treatments, for example, washing with water, treatment with acid, ultrasonic treatment, fungal/enzyme treatment and treatment with alkali (see Agusta et al., (2018) Journal of Japan Tappo 6, 641-49; Tye et al. (2013) Procedia Environmental Sciences 20, 328-335; Farah et al., 2014, BioResource 9(1), 938-951; Nik et al., (208), MCRJ Special Issue 4(2), 117-128; Zawati et al., (2015) Wood Research 60(1), 157-166; Harsono et al., (2015), Journal of Wood Science 62, 55-73; Rusdan (2002) Oil Palm Bulletin 44, 19-24); Rusdan et al., (2018) Journal of Tropical Forest Science 19(3), 121-126; ; Bahrin et al., (2012) Biorescources 7(2), 1784-1801; and Isroi et al., Molecules 17(12), 14995-15002).

With any pre-treatment process, it is necessary to balance the removal of the impurity, in this case, silica bodies, against the damage caused to the EFB feedstock by the pre-treatment process. The majority of these pre-treatments have been described in the context of a producing either sugar for bioethanol production, the production of furfural or the production of chemical pulps. In contrast, the present invention is primarily concerned with processes for producing man-made cellulosic fibers (regenerated cellulose) for the textiles industry, such as viscose, which are particularly sensitive to both the presence of silica and any fiber damage incurred during earlier processing steps. Thus, while the known processes may remove enough silica for the end applications for which they have been designed, the levels of silica which remain are still too high to be acceptable in the regenerated cellulose fiber textiles industry.

Therefore, it is clear that there is a need for pre-treatment processes for non-wood feedstock which is ultimately to be used in fiber manufacture, which remove high levels of silica without damaging the non-wood feedstock.

WO 2015/108409 A1 describes an integrated process for fractionation of oil palm empty fruit bunch (EFB) to obtain cellulosic solid, hemicellulosic sugars and high-purity lignin, and conversion of the cellulosic solid to ethanol by enzymatic hydrolysis and microbial fermentation.

### Summary of invention

Against this background, the present inventors have identified pre-treatment processes which are effective in removing silica bodies from non-wood feedstock, while avoiding causing significant damage to the cellulosic component of the feedstock.

The present invention is defined by the appended claims. In one aspect, the present invention provides a method for pre-treating non-wood feedstock comprising:
(a) washing non-wood feedstock;
(b) contacting the washed non-wood feedstock with an acid solution; and
(c) contacting the washed non-wood feedstock with an alkali solution;
wherein the method includes an additional washing step (d) between steps (b) and (c), as defined in appended claim 1.

Advantageously, the inventors have found that by carrying out the steps (a), (b), (c) and (d) this pre-treatment process results in a feedstock which contains very little silica while retaining its structural integrity and minimising damage to the cellulosic component of the feedstock. In particular, the inventors have surprisingly found that by combining a series of steps, each of which is carried out under conditions which are sufficiently mild to avoid unwanted structural damage, it is possible to remove effectively problematic silica bodies from the fibers of the feedstock. This is particularly surprising given the previous understanding in the industry that extreme and/or harsh conditions are required in order to remove these silica bodies.

Furthermore, the pre-treatment method of the present invention can be incorporated easily into existing saw dust/pin chip mills, organosolv and soda or kraft pulp mills. It is particularly advantageous for use in an integrated pulp mill *i.e* a mill in which the complete process from feedstock to end product is performed, because reactants from later stages in the process can be recycled back into the pre-treatment method, in particular step (b). This improves efficiency and minimises waste.

The present invention further provides Dissolving Pulp (DP) derived from non-wood empty fruit bunch (EFB) feedstock, which has a silica content of less than about 80 ppm. Advantageously, the low levels of silica present in the DP mean that it can be subsequently processed into regenerated cellulose fibers for use in the textiles industry to produce a high quality product. In particular, where silica is still present in the DP, it will cause issues with cellulose dissolution and clog the spinnerets which are subsequently used to draw the DP into fibers.

The present invention yet further provides Kraft Pulp (KP) derived from non-wood empty fruit bunch (EFB) feedstock, which has a silica content of less than about 600 ppm. Advantageously, the low levels of silica present in the KP mean that it can be subsequently processed into paper products without damaging the pulping machinery used. In particular, where silica is still present in the KP, it can lead to its deposition in the pulping machinery *(i.e.* sand deposits) which, as well as potentially damaging the machinery, can also lead to holes in the end product. The KP produced by the methods described herein does not suffer from these problems.

The inventors have found that the DP and KP obtained from feedstock which has been pre-treated according to the methods of the present invention has a quality which is equivalent to or better than that obtained using conventional wood feedstocks. It can also be obtained in a comparable yield.

### Detailed Description

The present invention is defined by the appended claims.

The term "Non-Process Element (NPE)" is used herein to refer to unwanted inorganic impurities other than silica and ash, such as metals including iron and calcium.

The first step in the pre-treatment process of the present invention is step (a) in which the non-wood feedstock is washed. This washing step is included first for the purpose of removing residual oils from the non-wood feedstock. Washing may be carried out using either water and/or steam. Preferably washing step (a) is performed at a temperature in the range from 80°C to 100°C. Where water is used in washing step (a), at the lower end of this temperature range, it will be appreciated that a mixture of water and steam is present, while at the upper end of the temperature range, steam is present. Preferably, the non-wood feedstock is mechanically agitated, preferably by gentle mechanical agitation, during step (a) of the method of the present invention. Preferably, the non-wood feedstock is agitated only to a small degree, such as that which may be achieved by passing the non-wood feedstock through a screw-type conveyor. The skilled person will be familiar with screw-type conveyors, an example of which is shown in Figure 11.

Prior to step (a) of the method of the present invention, the non-wood feedstock may have been subjected to process steps which are standard in the industry, for example shredding. Where the non-wood feedstock is shredded, preferably the resulting fibers have a length in the range from about 5 mm to about 100mm.

After the initial washing step (a), the washed non-wood feedstock is contacted with an acid solution in step (b) of the method. Contacting the non-wood feedstock with acid reduces the content of any residual metal impurities. In particular, it is effective in removing iron and calcium residues from the feedstock. Furthermore, without wishing to be bound be theory, it is believed that this acid treatment step is also crucial in the process of removing silica from the feedstock. As described previously, non-wood feedstock, in particular EFB feedstock, has a structure in which silica bodies are embedded in the surfaces of the fibers. Contacting the fibers with acid causes the fibers to shrink, which in turn, starts a process of displacing the silica bodies.

The acid solution comprises an acid and water. Any acid may be used to form the acid solution. Preferably the acid used is selected from the group consisting of sulfuric acid, hydrochloric acid, a solution of chlorine dioxide in water and mixtures thereof. As will be described later, a pulp mill typically includes a bleaching step. An advantage of the pre-treatment method of the present invention is that the acid used in step (b) of the pre-treatment method can be provided by acid used in a bleaching step being recycled directly into step (b) of the pre-treatment method, thus improving efficiency, minimising waste and cost production.

The acid is included in the acid solution of step (b) at a concentration in the range from about 0.2 to 5.0%. This ensures that the acid solution is sufficiently concentrated that the fibers of the non-wood feedstock shrink to facilitate removal of silica impurities but is dilute enough that unwanted damage to the feedstock, in particular to the cellulose in the feedstock, is minimised.

Preferably step (b) is carried out at pH in the range from 1 to 3.

Step (b) is carried out at a temperature in the range from about 80°C to about 100°C. It is preferable to perform step (b) at an elevated temperature because it increases the speed with which step (b) proceeds and so the efficiency of the process.

Where the non-wood feedstock from step (a) has been washed at an elevated temperature as described previously, also performing step (b) at an elevated temperature *(i.e.* a temperature in the range from about 80 to about 100°) improves efficiencies in the overall process as it avoids the need to include a step before step (b) in which the washed non-wood feed stock is cooled.

Step (b) is carried out for a time sufficient to achieve shrinkage of the fibers. Step (b) has a duration in the range from about 30 to about 60 minutes. The extent to which step (b) has proceeded can be monitored by measuring the content of the impurities which are to be removed, specifically ash residue, NPEs and silica. At the end of step (b), typically the silica content will have reduced by a small amount, while ash residue and NPEs will have been almost completely removed. A person skilled in the art will be familiar with suitable quality measurements.

In step (c) of the method of the present invention, the washed non-wood feedstock is contacted with an alkali solution. Contacting the feedstock with an alkali solution further assists in the removal of silica impurities. More specifically, contacting the feedstock with an alkali solution causes the fibers to swell which contributes towards removal of the silica from the feedstock.

Step (c) is carried out after step (a). Step (c) is performed after step (b). This is advantageous because, as will be described in more detail later, after pre-treatment, the non-wood feedstock is cooked to form a pulp. A preferred cooking step is performed under alkaline conditions and hence, if the pre-treatment method finishes with an alkaline step, it is already at a pH which is appropriate for the cooking step and thus the need for an additional neutralization step is avoided.

It is the combination of steps (b) and (c), which shrink and swell the fibers of the non-wood feedstock, respectively, which leads to effective removal of silica impurities.

The alkali solution used in step (c) comprises an alkali and water. Any alkali may be used to form the alkali solution but preferably the alkali is sodium hydroxide. Sodium hydroxide is preferred because, as described above, it is also used in the later cooking step described above directly after pre-treatment. By using the same alkali in step (c), the overall process efficiency is improved.

The alkali is included in the alkali solution of step (c) at a concentration in the range from about 0.2 to about 5.0%. This ensures that the alkali solution is sufficiently concentrated that the fibers of the non-wood feedstock swell to facilitate removal of silica impurities but is dilute enough that unwanted damage to the feedstock, in particular cellulose in the feedstock, is minimised.

Preferably step (c) is carried out at a pH in the range from 12 to 14.

Step (c) is carried out at a temperature in the range from about 80°C to about 100°C. It is preferable to perform step (c) at an elevated temperature because it increases the speed with which step (b) proceeds and so the efficiency of the process.

Where the non-wood feedstock from step (a) has been washed at an elevated temperature as described previously, also performing step (c) at an elevated temperature *(i.e.* a temperature in the range from about 80 to about 100°) improves efficiencies in the overall process as it avoids the need to include a step before step (c) in which the washed non-wood feed stock is cooled.

Step (c) is carried out for a time sufficient to achieve swelling of the fibers. Step (c) has a duration in the range from about 30 to about 60 minutes. The extent to which step (c) has proceeded can be monitored by measuring the content of silica which remains in the feedstock. At the end of step (c), typically the silica content will have reduced significantly. A person skilled in the art will be familiar with suitable quality measurements.

The pre-treatment method of the present invention includes a further washing step, step (d), between steps (b) and (c), irrespective of the order in which steps (b) and (c) are performed. This washing step is included for the primary purpose of removing metal and silica (typically fine silica) impurities which have been displaced from the non-wood fibers as a consequence of the earlier steps which have been performed. The washing of step (d) may be carried out using either water and/or steam. Preferably washing step (d) is performed at a temperature in the range from 80°C to 100°C. Where water is used in washing step (d), at the lower end of this temperature range, it will be appreciated that a mixture of water and steam is present, while at the upper end of the temperature range, steam is present. Preferably, the non-wood feedstock is mechanically agitated, preferably by gentle mechanical agitation, during step (a) of the method of the present invention. Preferably, the non-wood feedstock is agitated only to a small degree, such as that which may be achieved by passing the non-wood feedstock through a screw-type conveyor. The skilled person will be familiar with screw-type conveyors, an example of which is shown in Figure 11.

The method of the present invention may include a further washing step (e) after whichever of step (b) or step (c) is performed last. Where present, this additional washing step is included for the primary purpose of removing silica impurities. The washing of step (e) may be carried out using either water and/or steam. Preferably washing step (e) is performed at a temperature in the range from 80°C to 100°C. Where water is used in washing step (e), at the lower end of this temperature range, it will be appreciated that a mixture of water and steam is present, while at the upper end of the temperature range, steam is present. Preferably, the non-wood feedstock is mechanically agitated, preferably by gentle mechanical agitation, during step (a) of the method of the present invention. Preferably, the non-wood feedstock is agitated only to a small degree, such as that which may be achieved by passing the non-wood feedstock through a screw-type conveyor. The skilled person will be familiar with screw-type conveyors, an example of which is shown in Figure 11.

Once subjected to the pre-treatment method of the present invention, the non-wood feedstock is suitable for further processing to form a pulp which can then, in turn, serve as a raw material for either paper or in the production of regenerated cellulose, for example viscose, modal, lyocell or other MMC fibers.

The methods of the present invention can be carried out using standard apparatus found in standard pulp mills with which the person skilled in the art will be familiar. In particular, the pre-treatment method of the present invention is useful in an integrated pulp mill so that materials e.g. acid which is used in a bleaching step can be recycled into the pre-treatment methods of the present inventions.

Prior to further processing, the non-wood feedstock may be formed into bales. Alternatively, prior to further processing, the non-wood feedstock may be pelletized.

A person skilled in the art will be familiar with suitable methods for converting the pre-treated non-wood feedstock into pulp. In particular, there are two general methods which are used for cooking the feedstock, specifically a sulfate (Kraft) process and a pre-hydrolysis (PH) kraft process.

In a Kraft process, the pre-treated non-wood feedstock is mixed with a hot mixture, known as "white liquor" which comprises water, sodium hydroxide and sodium sulfite. Anthraquinone may be included as an accelerant to improve yields. During this process, lignin present in the feedstock are broken down and dissolved in the alkali. The remaining solid pulp, known as "brown stock" can be collected ready to be subjected to further processing steps. The combined liquids (the "black liquor") which contain lignin fragments, a small fraction of carbohydrates, sodium sulfate, sodium carbonate and other inorganic salts, can be removed and then burned to provide energy which is fed back into the cooking process.

The "brown pulp" obtained in the Kraft process is typically bleached in order to provide a pulp which has a high brightness. There are a number of different bleaching processes which may be used and the skilled person will be familiar with these An example of a suitable bleaching process is Elemental Chlorine Free (ECF) bleaching in which the brown pulp is contacted sequentially with peroxymonosulfuric acid (which can be produced by mixing sulfuric acid and hydrogen peroxide), chlorine dioxide, hydrogen peroxide and chlorine dioxide. Another example of a suitable bleaching process is Total Chlorine Free (TCF) bleaching in which the brown pulp is subjected to bleaching with ozone and hydrogen peroxide. In particular, TCF typically includes four or five different stages including both treatment with chelating agent and several bleaching stages such as bleaching with oxygen, alkaline extraction with hydrogen peroxide addition, peracetic acid bleaching and/or hydrogen peroxide bleaching with or without oxygen. TCF bleaching has the advantage that no chlorine is used and so no chlorine-containing byproducts are generated. The quality of the pre-treated non-wood feedstock obtained by the method of the present invention means that less energy is required in the bleaching step.

An advantage of the pre-treatment method of the present invention is that the acid used in such a bleaching step can be recycled back into step (b) of the pre-treatment method, thus reducing the amount of acid required for the overall process and reducing waste.

In a PH kraft process, the non-wood feedstock is first subjected to a water-based auto-hydrolysis process which removes hemicelluloses and some lignin. It is then cooked (kraft cooking) under alkaline conditions to remove the majority of lignin and a small fraction of remaining hemicellulose. Final multi-stage bleaching steps (e.g. ECF bleaching or TCF bleaching) are performed to increase the final pulp brightness. Anthraquinone can be included as an accelerant to improve yields in a PH kraft process.

Preferably the pre-treated non-wood feedstock obtained from the method of the present invention is cooked using a PH Kraft process.

In both cooking methods, the quality of the pulp which is obtained can be controlled by varying several parameters, specifically the H-factor, the P-factor, the Kappa number and Active Alkali%. In particular, by controlling these parameters, it is possible to control whether the pulp obtained is Dissolving Pulp (DP) or Kraft Pulp (KP).

Dissolving Pulp (DP) is a high grade pure cellulosic pulp which has a high level of brightness, a uniform molecular weight distribution and an open pore structure, rendering it highly reactive. DP is typically used in the production of regenerated cellulose.

Kraft Pulp (KP) is a pulp which contains both cellulose and hemicellulose. KP is typically used in the production of paper.

As will be appreciated by the person skilled in the art, these parameters have standard definitions. The H-factor is a kinetic model for the rate of delignification and depends on both temperature and time. The P-factor depends on the time and the temperature in a water-based medium. The Kappa number is a measure of the completeness of the process and gives an indication of the amount of lignin which remains in the pulp; it is measured as the amount of standard potassium permanganate solution that the pulp will consume. The Active Alkali % is the total concentration of alkaline constituents, except carbonates, present in the reaction as determined by titration of a sample of the white liquor with strong acid according to the procedure which is set out in SCAN-N-30.

Examples of suitable parameter ranges to obtain DP and KP are set out in Table 1 below.

**Table 1**

| **Parameter** | **KP** | **DP** |
|---|---|---|
| Active Alkali (AA)% | 15 to 20 | 15 to 20 |
| P factor (150-170°C)^{£} | NA | 1000-1300 |
| H factor (150 to 170°C)^{£} | 100 to 300 | 100 to 300 |
| Kappa* | 14 - 20 | 6 -10 |

| | | |
|---|---|---|
| *measured according to Tappi T236-om-06. ^{£}measured using standard digester computer software with which the skilled person will be familiar. | | |

As a consequence of the pre-treatment method of the present invention to which the non-wood feedstock has been subjected, the present invention provides DP and KP which has a very low impurity content.

It has also been found that, surprisingly, where a non-wood feedstock is treated according to the methods of the present invention prior to cooking, shorter cooking times are required. This means that less energy is required for the cooking process. It has further been found that non-wood feedstock treated according to the methods of the present invention requires less bleaching. In addition, as can be seen in Figure 10, in the subsequent bleaching of non-wood feedstock which has been treated according to the methods of the present invention, there is a significant reduction in the bleaching chemicals required, particularly where the non-wood feedstock is EFB feedstock where the consumption of chemicals is almost halved.

In particular, the DP and KP obtained using the pre-treatment method of the present invention meets the specifications as set out in Table 2 below.

**Table 2**

| **Parameter** | **KP** | **DP** |
|---|---|---|
| Silica / ppm | 400 to 600 | <80 |
| Fe / ppm | No specification | <10 |
| Ca / ppm | No specification | <75 |
| Ash / % | <0.35 | < 0.12 |
| Brightness (ISO) / %** | 89.5 | 90 |
| Viscosity / ml/g*** | 450 - 900 | 350 - 550 |

| | | |
|---|---|---|
| **Measured according to Tappi T525-om-06 **Measured according to Tappi T230-om-04 at 25°C | | |

The low silica content of the DP obtained using the methods of the present invention is particularly surprising given the previous issues which have been encountered in attempts to remove silica from a non-wood feedstock. This is particularly the case where the non-wood feedstock is EFB feedstock.

In this regard, the present invention provides dissolving pulp derived from non-wood feedstock which has a silica content of less than about 80 ppm.

Silica content can be determined according to the method set out in standard Tappi T 211-om-07.

Alternatively or in addition, the dissolving pulp derived from non-wood feedstock has a Fe content of about 10ppm or less.

Iron (Fe) content can be determined according to the method set out in standard Tappi T618-cm-01.

Alternatively or in addition, the dissolving pulp derived from non-wood feedstock has a Ca content of about 75 ppm or less.

Calcium content can be determined according to the method set out in standard Tappi T618-cm-01.

The presence of Fe and/or Ca impurities within the DP is undesirable because it affects subsequent steps in which cellulose is dissolved and ultimately leads to the need to increase the amounts of chemicals where are used in such steps.

Alternatively or in addition, the dissolving pulp derived from non-wood feedstock has an ash content of about 0.12% by weight or less.

The ash content can be determined according to the method set out in standard Tappi T322-om-07.

The present invention further provides kraft pulp derived from non-wood feedstock which has a silica content of less than about 600 ppm.

Alternatively or in addition, the kraft pulp derived from non-wood feedstock has an ash content of about 0.35% or less.

In particular, the present invention provides dissolving pulp derived from non-wood empty fruit bunch (EFB) which has a silica content of less than about 80 ppm.

Alternatively or in addition, the dissolving pulp derived from non-wood EFB has a Fe content of about 10ppm or less.

Alternatively or in addition, the dissolving pulp derived from non-wood EFB has a Ca content of about 75 ppm or less.

Alternatively or in addition, the dissolving pulp derived from non-wood EFB has an ash content of about 0.12% or less.

The present invention further provides kraft pulp derived from non-wood empty fruit bunch (EFB) which has a silica content of less than about 600 ppm.

Alternatively or in addition, the kraft pulp derived from non-wood empty fruit bunch (EFB) has an ash content of about 0.35% or less.

The DP of the present invention has a high brightness. Brightness is a measure of the amount of incident light reflected from the pulp under specified conditions as measured by the method set out in standard Tappi T525-om-06. The DP of the present invention preferably has a Brightness (ISO) of about 90% or greater.

The KP of the present invention has a high brightness. Brightness is a measure of the amount of incident light reflected from the pulp under specified conditions as measured by the method set out in standard Tappi T525-om-06. The KP of the present invention preferably has a Brightness (ISO) of about 90% or greater.

The dissolving pulp obtained by the methods of the present invention may be further processed to provide regenerated cellulose. The term "regenerated cellulose" is used herein to describe a class of materials manufactured by the conversion of natural cellulose from a non-wood feedstock, to a soluble cellulosic derivative and subsequent regeneration, typically forming either a fiber or a film. A person skilled in the art will be familiar with techniques for processing dissolving pulp to form regenerated cellulose. A first step in this further processing is typically to convert the dissolving pulp into cellulose dope. Where the end product is viscose textile fibers, in a next step, the cellulose dope is typically subjected to a xanthation in the presence of CS₂ and sodium hydroxide. Where the end product is Lyocell textile fibers, the cellulose dope is typically subjected to a N-methylmorpholine N-oxide (NMMO) reaction. In both cases, the product of the subsequent step can be extruded through spinnerets and regenerated to form the desired man-made fibers, e.g. viscose and/or lyocell textile fibers. It is also possible to produce other man-made cellulose (MMC) fibers. It is an attractive option for the textiles industry because it can be produced using significantly less water than e.g. cotton and the resultant material is highly breathable.

The kraft pulp obtained by the methods of the present invention may be further processed to provide paper products. The person skilled in the art will be familiar with techniques for forming a paper product from pulp. In particular, processes typically involve suspending the pulp in water and then machinery to flatten, dry and cut to form sheets and rolls.

The invention will now be further described by reference to the following figures and examples which are in no way intended to be limiting on the scope of the claims.

### Figures

Figure 1 is an illustration of the position of silica bodies within an EFB fiber;
Figure 2 is a block diagram illustrating a pre-treatment method of the present invention;
Figure 3(a) shows the silica content of non-wood EFB feedstock before and after the pre-treatment according to the method of the present invention and as compared to prior art techniques;
Figure 3(b) (for reference) shows the silica content of non-wood bamboo feedstock before and after the pre-treatment according to the method described herein and as compared to prior art techniques;
Figure 4(a) shows the ash content of non-wood EFB feedstock before and after pre-treatment according to the method of the present invention and as compared to prior art techniques;
Figure 4(b) (for reference) shows the ash content of non-wood bamboo feedstock before and after pre-treatment according to the method described herein and as compared to prior art techniques;
Figure 5 shows the silica contents of a non-wood EFB feedstock and (for reference) a non-wood bamboo feedstock before and after the pre-treatment methods of the present invention;
Figure 6 is an image of non-wood EFB KP produced by the method of the present invention;
Figure 7 is an image of non-wood EFB DP produced by the method of the present invention;
Figure 8 is a block diagram illustrating a process for producing paper products which includes the pre-treatment method of the present invention; and
Figures 9(a) is a block diagram illustrating a process for producing viscose which includes the pre-treatment of the present invention;
Figure 9(b) is a block diagram illustrating a process for producing lyocell which includes the pre-treatment of the present invention; and
Figure 10 shows the consumption of chlorine dioxide (ClO₂) during an ECF bleaching process performed on EFB feedstock treated according to the methods of the present invention as compared to hardwoods, specifically acacia crassicarpa (ACRA), Eucalyptus pellita (EPEL), Eucalyptus hybrid (EHYB);
Figure 11 shows a screw-type conveyor which may be used to move the non-wood feedstock from one stage to another in the method of the present invention;
Figure 12 shows the dates and times at which the feedstock was changed from a standard wood feedstock to a mixed EFB/wood feedstock in Example 3;
Figure 13 illustrates the productivity (H-factor) of the mill where the feedstock is changed from wood chip to mixed EFB/wood chip during the trial described in Example 3;
Figure 14 shows the oxygen charge consumed during bleaching in the mill described in Example 3;
Figure 15 shows the alkali charge consumed during bleaching in the mill described in Example 3;
Figure 16 shows the silica content of bleached kraft pulps obtained from the mixed feedstock as described in Example 3; and
Figure 17 illustrates the dirt spot/count of bleached kraft pulps obtained from the mixed feedstock as described in Example 3.

### Examples

### Example 1 - non-wood EFB feedstock

Approximately 100kg of non-wood EFB which had been processed so that it was free from kernel, palm seed and mud was obtained from Asian Agri (RGE palm oil business) and was passed into a shredder and washer to obtain EFB feedstock having a fiber length in the range from 5 to 100mm.

The silica and ash residue contents of the non-wood EFB were measured according to Tappi T618-cm-01. The results are shown in Figures 3(a) and 4(a).

The non-wood EFB feedstock was then washed using a mixture of water and steam at a temperature in the range from 80 to 100°C in a drum washer. The EFB feedstock was moved towards the next treatment step by screw conveyor (which provides a small degree of mechanical agitation). The washing step was carried out for a duration of 30 to 60 mins. The washed EFB feedstock was then passed to a vessel which contained-acid solution in sufficient liquor ratio (7 to 10) having a pH in the range from 1 to 3 and at a temperature in the range from 80 to 100°C. After 30 to 60 mins, the EFB feedstock was removed from the acid-containing vessel and passed to a drum washer where it was washed using a mixture of water and steam at a temperature in the range from 80 to 100°C. After 30 to 60 mins, the washed and acid-treated EFB feedstock was passed to a vessel which contained alkali solution in sufficient liquor ratio (7 to 10) having a pH in the range from 12 to 14 and at a temperature in the range from 80 to 100°C. After 30 to 60 mins, the EFB was removed from the alkali-containing vessel and passed to a drum washer where it was washed using a mixture of water and steam at a temperature in the range from 80 to 100°C. The pre-treated EFB feedstock was moved toward the next step by a screw conveyor (which provides a small degree of mechanical agitation).

The silica and ash residue contents of the pre-treated EFB feedstock were measured according to Tappi T618-cm-01 and are illustrated in Figures 3(a) and 4(b).

The pre-treated EFB feedstock was then cooked under prehydrolysis kraft (P- factor 1000 to 1300)/kraft for both DP and KP. Active alkali was used in an amount in the range from 15 to 20% and the H factor was in the range from about 100 to 300 (see Table 1). The target specifications for chemical pulps (DP & KP), as set out in Table 2 were achieved.

### Example 2 (reference) - non-wood bamboo feedstock

Approximately 5kg of non-wood bamboo bark was chipped and passed through a mesh screen of size 7 to 13 mm to form bamboo chips of a standard size

The silica and ash residue contents of the non-wood bamboo were measured according to Tappi T618-cm-01. The results are shown in Figures 3(b) and 4(b).

The non-wood bamboo feedstock was then washed using a mixture of water and steam at a temperature in the range from 80 to 100°C in a drum washer. The bamboo feedstock was moved towards the next treatment step by a conveyor belt. The washing step was carried out for a duration of 30 to 60 mins. The washed bamboo feedstock was then passed to a vessel which contained acid solution in sufficient liquor ratio (4 to 7) having a pH in the range from 1 to 3 and at a temperature in the range from 80 to 100°C. After 30 to 60 mins, the bamboo feedstock was removed from the acid-containing vessel and passed to a drum washer where it was washed using a mixture of water and steam at a temperature in the range from 80 to 100°C. After 30 to 60 mins, the washed and acid-treated bamboo feedstock was passed to a vessel which contained alkali solution in sufficient liquor ratio (4 to 7) having a pH in the range from 12 to 14 and at a temperature in the range from 80 to 100°C. After 30 to 60 mins, the bamboo feedstock was removed from the alkali-containing vessel and passed to a drum washer where it was washed using a mixture of water and steam at a temperature in the range from 80 to 100°C. The pre-treated bamboo feedstock was moved toward the next step by a conveyor belt.

The silica and ash residue contents of the pre-treated bamboo feedstock were measured according to Tappi T618-cm-01 and are illustrated in Figures 3(b) and 4(b).

The pre-treated bamboo feedstock was then cooked under prehydrolysis kraft (P- factor 500 to 800)/ kraft for both DP and KP. Active alkali was used in an amount in the range from 15 to 20 % and the H factor was in the range from about 500 to 700. The target specification for chemical pulps (DP & KP), as set out in Table 2 earlier was achieved.

### Example 3 - EFB feedstock Mill trial

Standard wood feedstock was replaced with a mixed wood feedstock comprising 5 to 10% by weight EFB feedstock in a running mill which processes 35 tonnes of feedstock per day.

Various outputs were monitored as summarised below. The process to which the mixed EFB feedstock was subjected included the pre-treatment method of the present invention.

Figure 12 illustrates the point at which the feedstock was altered to comprise 5 to 10% by weight of EFB feedstock. It is clear from Figure 13 that a higher cooking productivity (as evidenced by a lower H-factor) was observed for the same level of alkali charge and kappa number where the feed was changed to a mixed EFB feedstock. With reference to Figures 14 and 15, it is also clear that the consumption of chemicals in the bleaching step was reduced - both the oxygen and alkali charges were reduced and the total charge of ClO₂ was also reduced (47.3 kg for pure wood feedstock vs. 46.2kg for mixed EFB/wood feedstock).

In addition to these reductions in both chemical consumption and energy required, advantageously, it has been found that the quality of the final bleached pulps were maintained.

In particular, the pulps obtained had the following properties:

**Table 3**

| **Parameter** | **Value** |
|---|---|
| Brightness | 89.5% |
| Viscosity | 631 dm³/kg |
| Freeness | 536 ml CSF |
| Dirt | 6mm²/m² |
| Silica content | 432 mg/l |

The end product in the mill trial described in Example 3 was a paper product. Where the feedstock was changed from pure wood to a mixture of EFB and wood and the process included the pre-treatment method of the present invention, it was surprisingly found that the end paper product had excellent properties, specifically a tensile strength of 70 Nm/g and a bulk density of 1.39 cm³/g. The paper also demonstrated high performance in both drainability and runnability.

Overall, in replacing the wood feedstock with a mixed EFB/wood feedstock and including the pre-treatment method of the present invention, it was possible to produce products having the required excellent properties while reducing energy consumption by approximately 10%.

## Claims

1. A method for pre-treating non-wood empty fruit bunch (EFB) feedstock comprising:
(a) washing non-wood empty fruit bunch (EFB) feedstock;
(b) contacting the washed non-wood empty fruit bunch (EFB) feedstock with an acid solution at a temperature in the range from 80 to 100°C for a duration of 30 to 60 minutes; and
(c) contacting the washed non-wood feedstock with an alkali solution at a temperature in the range from 80 to 100°C for a duration of 30 to 60 minutes;
wherein the method includes an additional washing step (d) between steps (b) and (c); and wherein step (b) is performed before step (c), and
wherein the method for pre-treating provides non-wood feedstock suitable to be cooked to produce a dissolving pulp (DP) or a kraft pulp (KP).

2. A method for producing dissolving pulp (DP) from non-wood empty fruit bunch (EFB) feedstock comprising:
(i) pre-treating non-wood empty fruit bunch (EFB) feedstock comprising:
(a) washing non-wood empty fruit bunch (EFB) feedstock;
(b) contacting the washed non-wood empty fruit bunch (EFB) feedstock with an acid solution at a temperature in the range from 80 to 100°C for a duration of 30 to 60 minutes; and
(c) contacting the washed non-wood feedstock with an alkali solution at a temperature in the range from 80 to 100°C for a duration of 30 to 60 minutes;
wherein the method includes an additional washing step (d) between steps (b) and (c); and wherein step (b) is performed before step (c); and
(ii) cooking the pre-treated non-wood empty fruit bunch (EFB) feedstock to produce DP.

3. A method for producing kraft pulp (KP) from non-wood empty fruit bunch (EFB) feedstock comprising:
(i) pre-treating non-wood empty fruit bunch (EFB) feedstock comprising:
(a) washing non-wood empty fruit bunch (EFB) feedstock;
(b) contacting the washed non-wood empty fruit bunch (EFB) feedstock with an acid solution at a temperature in the range from 80 to 100°C for a duration of 30 to 60 minutes; and
(c) contacting the washed non-wood feedstock with an alkali solution at a temperature in the range from 80 to 100°C for a duration of 30 to 60 minutes;
wherein the method includes an additional washing step (d) between steps (b) and (c); and wherein step (b) is performed before step (c); and
(ii) cooking the pre-treated non-wood empty fruit bunch (EFB) feedstock to produce KP.

4. A method according to any preceding claim, wherein in step (a), the non-wood empty fruit bunch (EFB) feedstock is washed using water and/or steam.

5. A method according to any preceding claim, wherein in step (d), the non-wood empty fruit bunch (EFB) feedstock is washed using water and/or steam.

6. A method according to any preceding claim which further comprises:
(e) washing the product obtained after steps (a) to (d).

7. A method according to any preceding claim, wherein acid is included in the acid solution of step (b) at a concentration in the range from 0.2 to 5.0% and/or wherein alkali is included in the alkali solution of step (c) at a concentration in the range from 0.2 to 5.0%.

8. Dissolving pulp derived from non-wood empty fruit bunch (EFB) feedstock obtainable by the method of claim 2 which has a silica content of less than 80 ppm.

9. Dissolving pulp according to claim 8 which has a Fe content of 10ppm or less.

10. Dissolving pulp according to any one of claims 8 or 9, which has a Ca content of 75 ppm or less.

11. Dissolving pulp according to any one of claims 8 to 9 which has an ash content of 0.12% or less.

12. Kraft pulp derived from non-wood empty fruit bunch (EFB) feedstock obtainable by the method of claim 3 which has a silica content of less than 600 ppm.

13. Kraft pulp according to claim 12, which has an ash content of 0.35% by weight or less.

14. Use of Dissolving Pulp (DP) as defined in claims 8 to 11, in the manufacture of cellulosic fibers.

15. Use of Kraft Pulp (KP) as defined in claim 12 or claim 13, in the manufacture of paper.

## Patentansprüche

1. Verfahren zum Vorbehandeln nicht-holzartigen leeren Fruchtbündel-(EFB)-Rohmaterials, umfassend:
(a) Waschen nicht-holzartigen leeren Fruchtbündel-(EFB)-Rohmaterials;
(b) Kontaktieren des gewaschenen nicht-holzartigen leeren Fruchtbündel-(EFB)-Rohmaterials mit einer Säurelösung bei einer Temperatur in dem Bereich von 80 bis 100 °C für eine Zeitdauer von 30 bis 60 Minuten; und
(c) Kontaktieren des gewaschenen nicht-holzartigen Rohmaterials mit einer Alkalilösung bei einer Temperatur in dem Bereich von 80 bis 100 °C für eine Zeitdauer von 30 bis 60 Minuten;
wobei das Verfahren einen zusätzlichen Waschschritt (d) zwischen den Schritten (b) und (c) umfasst;
und wobei Schritt (b) vor Schritt (c) durchgeführt wird, und
wobei das Verfahren zum Vorbehandeln nicht-holzartiges Rohmaterial bereitstellt, welches dazu geeignet ist, gekocht zu werden, um einen Chemiezellstoff (DP) oder einen Kraftzellstoff (KP) zu erzeugen.

2. Verfahren zum Erzeugen von Chemiezellstoff (DP) aus nicht-holzartigem leerem Fruchtbündel-(EFB)-Rohmaterial, umfassend:
(i) Vorbehandeln nicht-holzartigen leeren Fruchtbündel-(EFB)-Rohmaterials, umfassend:
(a) Waschen nicht-holzartigen leeren Fruchtbündel-(EFB)-Rohmaterials;
(b) Kontaktieren des gewaschenen nicht-holzartigen leeren Fruchtbündel-(EFB)-Rohmaterials mit einer Säurelösung bei einer Temperatur in dem Bereich von 80 bis 100 °C für eine Zeitdauer von 30 bis 60 Minuten; und
(c) Kontaktieren des gewaschenen nicht-holzartigen Rohmaterials mit einer Alkalilösung bei einer Temperatur in dem Bereich von 80 bis 100 °C für eine Zeitdauer von 30 bis 60 Minuten;
wobei das Verfahren einen zusätzlichen Waschschritt (d) zwischen den Schritten (b) und (c) umfasst;
und wobei Schritt (b) vor Schritt (c) durchgeführt wird, und
(ii) Kochen des nicht-holzartigen leeren Fruchtbündel-(EFB)-Rohmaterials, um DP zu erzeugen.

3. Verfahren zum Erzeugen von Kraftzellstoff (KP) aus nicht-holzartigem leerem Fruchtbündel-(EFB)-Rohmaterial, umfassend:
(i) Vorbehandeln nicht-holzartigen leeren Fruchtbündel-(EFB)-Rohmaterials, umfassend:
(a) Waschen nicht-holzartigen leeren Fruchtbündel-(EFB)-Rohmaterials;
(b) Kontaktieren des gewaschenen nicht-holzartigen leeren Fruchtbündel-(EFB)-Rohmaterials mit einer Säurelösung bei einer Temperatur in dem Bereich von 80 bis 100 °C für eine Zeitdauer von 30 bis 60 Minuten; und
(c) Kontaktieren des gewaschenen nicht-holzartigen Rohmaterials mit einer Alkalilösung bei einer Temperatur in dem Bereich von 80 bis 100 °C für eine Zeitdauer von 30 bis 60 Minuten;
wobei das Verfahren einen zusätzlichen Waschschritt (d) zwischen den Schritten (b) und (c) umfasst;
und wobei Schritt (b) vor Schritt (c) durchgeführt wird, und
(ii) Kochen des nicht-holzartigen leeren Fruchtbündel-(EFB)-Rohmaterials, um KP zu erzeugen.

4. Verfahren nach einem vorhergehenden Anspruch, wobei in Schritt (a) das nicht-holzartige leere Fruchtbündel-(EFB)-Rohmaterial unter Verwendung von Wasser und/oder Dampf gewaschen wird.

5. Verfahren nach einem vorhergehenden Anspruch, wobei in Schritt (d) das nicht-holzartige leere Fruchtbündel-(EFB)-Rohmaterial unter Verwendung von Wasser und/oder Dampf gewaschen wird.

6. Verfahren nach einem vorhergehenden Anspruch, welches ferner umfasst:
(e) Waschen des Produkts, welches nach den Schritten (a) bis (d) erhalten wird.

7. Verfahren nach einem vorhergehenden Anspruch, wobei in der Säurelösung aus Schritt (b) eine Säure mit einer Konzentration in dem Bereich von 0,2 bis 5,0 % umfasst ist, und/oder wobei in der Alkalilösung aus Schritt (c) ein Alkali mit einer Konzentration in dem Bereich von 0,2 bis 5,0 % umfasst ist.

8. Chemiezellstoff, welcher von nicht-holzartigem leerem Fruchtbündel-(EFB)-Rohmaterial stammt, welches durch das Verfahren nach Anspruch 2 erhaltbar ist, und welcher einen Siliziumoxidgehalt von weniger als 80 ppm aufweist.

9. Chemiezellstoff nach Anspruch 8, welcher einen Fe-Gehalt von 10 ppm oder weniger aufweist.

10. Chemiezellstoff nach einem der Ansprüche 8 oder 9, welcher einen Ca-Gehalt von 75 ppm oder weniger aufweist.

11. Chemiezellstoff nach einem der Ansprüche 8 bis 9, welcher einen Aschegehalt von 0,12 % oder weniger aufweist.

12. Kraftzellstoff, welcher von nicht-holzartigem leerem Fruchtbündel-(EFB)-Rohmaterial stammt, welches durch das Verfahren nach Anspruch 3 erhaltbar ist, und welcher einen Siliziumoxidgehalt von weniger als 600 ppm aufweist.

13. Kraftzellstoff nach Anspruch 12, welcher einen Aschegehalt von 0,35 Gew.-% oder weniger aufweist.

14. Verwendung eines Chemiezellstoffs (DP) nach einem der Ansprüche 8 bis 11 in der Herstellung von Zellulosefasern.

15. Verwendung eines Kraftzellstoffs (KP) nach Anspruch 12 oder Anspruch 13 in der Herstellung von Papier.

## Revendications

1. Procédé pour prétraiter une matière première de rafle (EFB) non ligneuse comportant :
(a) le lavage de la matière première de rafle (EFB) non ligneuse ;
(b) la mise en contact de la matière première de rafle (EFB) non ligneuse lavée avec une solution acide à une température dans la plage de 80 à 100 °C pendant une durée de 30 à 60 minutes ; et
(c) la mise en contact de la matière première non ligneuse lavée avec une solution alcaline à une température dans la plage de 80 à 100 °C pendant une durée de 30 à 60 minutes ;
dans lequel le procédé inclut une étape de lavage (d) supplémentaire entre les étapes (b) et (c) ; et dans lequel l'étape (b) est réalisée avant l'étape (c), et
dans lequel le procédé pour prétraiter fournit une matière première non ligneuse adaptée pour être cuite pour produire une pâte à dissoudre (DP) ou une pâte kraft (KP).

2. Procédé pour produire de la pâte à dissoudre (DP) à partir d'une matière première de rafle (EFB) non ligneuse comportant :
(i) le prétraitement d'une matière première de rafle (EFB) non ligneuse comportant :
(a) le lavage de la matière première de rafle (EFB) non ligneuse ;
(b) la mise en contact de la matière première de rafle (EFB) non ligneuse lavée avec une solution acide à une température dans la plage de 80 à 100 °C pendant une durée de 30 à 60 minutes ; et
(c) la mise en contact de la matière première non ligneuse lavée avec une solution alcaline à une température dans la plage de 80 à 100 °C pendant une durée de 30 à 60 minutes ;
dans lequel le procédé inclut une étape de lavage (d) supplémentaire entre les étapes (b) et (c) ; et dans lequel **l'étape** (b) est réalisée avant **l'étape** (c) ; et
(ii) la cuisson de la matière première de rafle (EFB) non ligneuse prétraitée pour produire la DP.

3. Procédé pour produire de la pâte kraft (KP) à partir d'une matière première de rafle (EFB) non ligneuse comportant :
(i) le prétraitement d'une matière première de rafle (EFB) non ligneuse comportant :
(a) le lavage de la matière première de rafle (EFB) non ligneuse ;
(b) la mise en contact de la matière première de rafle (EFB) non ligneuse lavée avec une solution acide à une température dans la plage de 80 à 100 °C pendant une durée de 30 à 60 minutes ; et
(c) la mise en contact de la matière première non ligneuse lavée avec une solution alcaline à une température dans la plage de 80 à 100 °C pendant une durée de 30 à 60 minutes ;
dans lequel le procédé inclut une étape de lavage (d) supplémentaire entre les étapes (b) et (c) ; et dans lequel **l'étape** (b) est réalisée avant **l'étape** (c) ; et
(ii) la cuisson de la matière première de rafle (EFB) non ligneuse prétraitée pour produire la KP.

4. Procédé selon une quelconque revendication précédente, dans lequel, à l'étape (a), la matière première de rafle (EFB) non ligneuse est lavée à l'aide d'eau et/ou de vapeur.

5. Procédé selon une quelconque revendication précédente, dans lequel, à l'étape (d), la matière première de rafle (EFB) non ligneuse est lavée à l'aide d'eau et/ou de vapeur.

6. Procédé selon une quelconque revendication précédente qui comporte en outre :
(e) le lavage du produit obtenu après les étapes (a) à (d).

7. Procédé selon une quelconque revendication précédente, dans lequel l'acide est inclus dans la solution acide de l'étape (b) à une concentration dans la plage de 0,2 à 5,0 % et/ou dans lequel l'alcali est inclus dans la solution alcaline de l'étape (c) à une concentration dans la plage de 0,2 à 5,0 %.

8. Pâte à dissoudre dérivée d'une matière première de rafle (EFB) non ligneuse pouvant être obtenue par le procédé selon la revendication 2 qui a une teneur en silice inférieure à 80 ppm.

9. Pâte à dissoudre selon la revendication 8 qui a une teneur en Fe de 10 ppm ou moins.

10. Pâte à dissoudre selon l'une quelconque des revendications 8 ou 9**,** qui a une teneur en Ca de 75 ppm ou moins.

11. Pâte à dissoudre selon l'une quelconque des revendications 8 à 9 qui a une teneur en cendres de 0,12 % ou moins.

12. Pâte kraft dérivée d'une matière première de rafle (EFB) non ligneuse pouvant être obtenue par le procédé selon la revendication 3 qui a une teneur en silice inférieure à 600 ppm.

13. Pâte kraft selon la revendication 12, qui a une teneur en cendres de 0,35 % en poids ou moins.

14. Utilisation de pâte à dissoudre (DP) telle que définie dans les revendications 8 à 11, dans la fabrication de fibres cellulosiques.

15. Utilisation de pâte kraft (KP) telle que définie dans la revendication 12 ou revendication 13, dans la fabrication de papier.
